

July 21, 1925.

1,546,796

M. SAUNDERS

APPARATUS AND PROCESS FOR CASTING STEEL INGOTS

Filed Jan. 3, 1924



Fig. 3



Fig. 8



Fig. 9



Fig. 4



Inventor  
M. Saunders

Greene and Bowd

Attorneys

Fig.

## UNITED STATES PATENT OFFICE.

MALCOLM SAUNDERS, OF CANTON, OHIO.

## APPARATUS AND PROCESS FOR CASTING STEEL INGOTS.

Application filed January 3, 1924. Serial No. 684,119.

*To all whom it may concern:*

Be it known that I, MALCOLM SAUNDERS, a citizen of the United States, residing at Canton, in the county of Stark and State of Ohio, have invented certain new and useful Improvements in Apparatus and Processes for Casting Steel Ingots, of which the following is a specification.

This invention relates to the casting of steel ingots and has more especial reference to an apparatus and process for perfecting the ingots and eliminating the formation of defects known as "piping," which commonly occur in the pouring of ingots due to the gas bubbles which rise through the molten metal and to the shrinkage of the metal.

It is well known that these defective portions of the ingots must be chipped or ground out when the steel is rolled, resulting in a loss of from five per cent (5%) to as high as forty per cent (40%) of the steel and requiring considerable time and labor which necessarily increases the cost of the production of steel.

It is well known common practice in steel mills to use "brick tops" or "hot tops" upon the ingot molds in an attempt to eliminate these defects in the ingots, but even with the use of such devices, only a portion of the impressions in the ingots is avoided, and steel rolled from the two ends of an ingot formed in the ordinary manner will have different characteristics.

The objects of the present invention are to provide an apparatus and process for casting ingots, which includes a hollow plunger adapted to be supported at the upper end of an ingot mold and having an upwardly tapered interior designed to have a wedging action upon the upper end of the ingot while it is still hot, in order to eliminate any piping in the same, a pair of perforated plugs, one of which is preferably formed of fire clay or other refractory material and the other of cast iron, being placed upon the top of the poured metal within the hollow plunger to permit the gas to pass through the same.

The above and other objects may be attained by constructing the apparatus in the manner illustrated in the accompanying drawing, in which—

Figure 1 is a vertical sectional view of

an ingot mold provided with the improved plunger, showing the same in the initial position just after the steel has been poured;

Fig. 2, a similar view showing the same after the plunger has been lowered;

Fig. 3, a view similar to Figs. 1 and 2, showing a portion of the stripping machine in the act of removing the finished ingot from the mold;

Fig. 4, a bottom plan view of the brake band;

Fig. 5, an enlarged sectional view through a portion of the hollow plunger and ingot mold, showing the brake band operating lever in position to lock the band around the plunger;

Fig. 6, a detail sectional view on the line 6—6, Fig. 5;

Fig. 7, a plan view of the safety plug;

Fig. 8, a similar view of the fire brick plug; and

Fig. 9, a vertical sectional view of a slightly modified form of the apparatus adapted for "large top molds."

Similar numerals refer to similar parts throughout the drawing.

Referring to the construction shown in Figs. 1 to 8 inclusive, the ingot mold 1 may be of any usual "large bottom" construction, either plain or fluted.

The interior of the upper end portion of the mold indicated at 2 is round, and preferably machined for a sufficient distance from the top to accommodate the hollow plunger 3 which may be formed of cast iron and is machined to provide a sliding fit of the same within the upper end of the mold.

This plunger is provided with the central, upwardly tapered opening 4 and with the enlarged annular head 5 at its upper end upon which are provided lugs 6 for raising or lowering the plunger. The lower edge of the plunger is bevelled or rounded as shown at 6' to provide easy passage of the same through the metal and also to give the proper shape to the ingots.

The plunger may be held in raised position, as shown in Fig. 1, by means of a brake band 7 which may be in the form of a two part steel ring, as shown in Fig. 4. The two halves of the ring may be hinged together at one end as shown at 8, the free ends being provided with the angular por-

tions 9 and 10 respectively, a web 11 being formed upon the portion 10.

A bolt 12 is extended through the angular portions 9 and 10 and beneath the web 11, a 5 heavy coil spring 13 being located around the same between the side of the angular portion 10 and the head 15 of the bolt, tending to urge the halves of the brake band toward each other.

10 The lever 16 may be pivoted upon the bolt 12 and provided with the wedge portion 17, intermediate its extremities, arranged to separate the halves of the ring against the action of the spring 13, when it is desired to 15 release the tension upon the plunger.

In operating the apparatus to pour an ingot, the plunger is raised into the position shown in Fig. 1, the lever 16 of the brake band being raised to permit the brake band 20 to tightly grip the plunger and hold the same supported in this position.

The steel is then poured into the ingot and up into the plunger to about the height shown in Fig. 1. The perforated plug 18, 25 which may be of fire brick or similar material, or which may be in the form of a mat of straw or the like, is then inserted through the top of the plunger and placed upon the top of the molten steel and the perforated 30 safety plug 19 which may be of cast iron, steel or the like, is then inserted through the open upper end of the plunger, a wire 19<sup>a</sup> being preferably looped through the perforations of the plug, whereby the same may 35 be pulled to the top of the opening and held wedged therein by twisting the wire around a small rod 19<sup>b</sup>. The plug 18 may be heated before it is placed upon the metal, to assist in retaining the heat at the top of the 40 ingot.

It will be noted that each of these plugs is provided upon the diametrically opposite sides with the flat faces 20 to permit their being easily inserted through the reduced 45 top of the plunger and in placing these plugs upon the top of the molten steel, the flat faces of the two plugs should be staggered as shown in the drawings, in order to completely close the plunger, excepting for 50 the perforations in the plungers, which permit the gases from the molten steel to escape through the top of the plunger.

The metal will immediately start to freeze around the outside, checking the gases from 55 escaping. The brake band is then released by throwing the lever down, the wedge 17 thereon forcing the halves of the ring apart, against the action of the spring 13, permitting the plunger, which, of course, will be 60 of considerable weight, to descend in the manner shown in Fig. 2, the conical interior of the plunger forcing in the sides of the ingot at the top thereof, breaking the frozen crust upon the ingot and closing the central 65 portion of the ingot before the same has

hardened, an equal pressure being exerted upon all sides of the ingot, forcing the metal toward the center and the gases out of the top, thus removing any piping which may otherwise form in the ingot.

70 After the ingot has cooled, it may be removed from the mold by the usual stripper machine, indicated generally at 21, the jaws 22 thereof engaging the lugs at the top of the ingot mold in the usual manner, 75 while the plunger 23 is moved down through the open plunger and forces the ingot through the open bottom of the mold.

A modification of the invention is shown in Fig. 9, in which a "large top" mold 1<sup>a</sup> is 80 provided with the improved apparatus. A collar 24 provided with a depending flange 25 at its inner edge, is placed upon the top of the mold, the flange 25 extending down into the top thereof. This collar receives 85 the open plunger 3 which may be of the same construction as above described and operated in the same manner.

It will be seen that steel poured in accordance with the above described process, 90 and using an apparatus of the character described and illustrated, will be free from piping. Since the open plunger has considerable weight, it will be evident that as the ingot is cooling, an even pressure will 95 be applied to the sides of the cooling steel at the upper portion thereof, squeezing the mass toward the center and eliminating any piping while the perforations in the plugs will permit the gases to escape during the 100 time the hot steel is being squeezed together, thus producing a solid mass and eliminating the imperfections in the finished ingot.

It will also be seen that this device also 105 accomplishes the purposes of the usual brick top as it will retain the heat of the ingot at the top until the bottom of the ingot has cooled sufficiently to solidify, while at the same time sufficient pressure is exerted upon the sides of the upper portion of the ingot 110 to weld the same into a solid mass.

It will of course be understood that when the improved apparatus is used upon "large top" molds, it will be necessary to remove the plunger and collar before the ingot can 115 be stripped from the mold.

I claim:—

1. The improved method of forming ingots from molten metal which consists in retaining the heat in the upper portion of the ingot until the lower portion has solidified and applying sufficient downward pressure to the top and sides of the upper portion of the ingot to weld all portions of the ingot into a solid mass.

120 2. The improved method of forming ingots from molten metal which consists in downwardly compressing the top and sides of the upper portion of the ingot while the same is still hot and in covering the top of 125

the ingot with a perforated cover of refractory material to permit the escape of gases during said compression.

3. The improved method of forming ingots from molten metal which consists in lowering a plunger having a conical central opening around the upper portion of the metal to exert an equal pressure upon all sides and the top of the metal to press the same toward the center.

4. An ingot casting apparatus including an open top mold, a plunger slidably fitting within the top of the mold and having an upwardly tapered, central opening, and a brake band resting upon the top of the mold and engaging the plunger to hold the same in raised position.

5. An ingot casting apparatus including an open top mold, a plunger slidably fitting within the top of the mold and having an upwardly tapered, central opening the lower end of which is of substantially the same cross sectional area as the mold, and means for holding the plunger in any desired vertical position.

6. An ingot casting apparatus including an open top mold, a plunger slidably fitting within the top of the mold and having an upwardly tapered, central opening, and a brake band comprising a two part hinged ring surrounding the plunger and resting upon the top of the mold, and spring means for drawing the ring together around the plunger.

35 7. An ingot casting apparatus including an open top mold, a plunger slidably fitting within the top of the mold and having an upwardly tapered, central opening, a brake band comprising a two part hinged ring surrounding the plunger and resting upon the top of the mold, spring means for drawing the ring together around the plunger, and means for releasing the brake band to permit the plunger to descend.

45 8. An ingot casting apparatus including an open top mold, a plunger slidably fitting within the top of the mold and having an upwardly tapered, central opening, a brake band comprising a two part hinged ring surrounding the plunger and resting upon the top of the mold, spring means for draw-

ing the ring together around the plunger, and means for releasing the brake band to permit the plunger to descend, said releasing means being designed to permit any desired drop of the plunger.

9. An ingot casting apparatus including an open top mold, a plunger slidably fitting within the top of the mold and having an upwardly tapered central opening and means for detachably holding the plunger in any desired vertical position, the engaging faces of the mold and plunger being finished to provide a close fit in order to prevent molten metal from entering between the mold and plunger and means for permitting gases to escape from the ingot during the operation of the plunger.

10. An ingot casting apparatus including an open top mold, the inner, upper edge of which is beveled and an open plunger slidably fitting within the top of the mold.

11. An ingot casting apparatus including an open top mold, a plunger slidably fitting within the top of the mold and having an upwardly tapered, central opening, and a perforated plug adapted to be placed through the top of the plunger upon the metal.

12. An ingot casting apparatus including an open top mold, a plunger slidably fitting within the top of the mold and having an upwardly tapered, central opening, and a beveled lower edge, and means for holding the plunger in any desired vertical position.

13. An ingot casting apparatus including an open top mold, a plunger slidably fitting within the top of the mold and having an upwardly tapered, central opening, a perforated fire clay plug adapted to be placed through the top of the plunger upon the metal and a perforated metal plug adapted to be placed through the top of the plunger and supported therein.

14. An ingot casting apparatus including an open top mold, and means at the top of the mold for wedging the upper portion of a hot ingot downward uniformly upon all sides.

In testimony that I claim the above, I have hereunto subscribed my name.

MALCOLM SAUNDERS.